

1

2,820,765

## THICKENED LUBRICANTS

Everett C. Hughes, Shaker Heights, and Ernest C. Milberger, Maple Heights, Ohio, assignors to The Standard Oil Company, Cleveland, Ohio, a corporation of Ohio

No Drawing. Application October 6, 1954  
Serial No. 460,760

4 Claims. (Cl. 252—25)

This invention relates to an aerogel grease of good high temperature stability and water resistance.

While the word "grease" has usually been employed to describe an oil thickened with a soap, it is here used in a broader sense to include any thickened lubricant.

It is generally known that soap-base greases break down at high temperatures, of the order of 300 to 400° F. This breakdown is accompanied by an irreversible change in the grease structure, so that upon cooling the grease is observed to have lost its grease-like characteristics. The aerogel greases usually are far superior to the soap-base greases in stability at high temperatures as the following table shows:

TABLE I

| Soap or other thickener | Appearance at 400° F. | Appearance after cooling                                   |
|-------------------------|-----------------------|------------------------------------------------------------|
| Aluminum                | Very gummy and soft.  | Hard and lumpy.                                            |
| Lithium                 | Liquid                | Do.                                                        |
| Calcium                 | do                    | Hard—separation of soap.                                   |
| Sodium                  | do                    | Solidifies hard mass.                                      |
| Do                      | do                    | Soupy                                                      |
| Sodium-calcium          | do                    | Complete separation of oil+soap.                           |
| Silica aerogel          | Unchanged             | Unchanged except somewhat thinner.                         |
| Do                      | do                    | Unchanged, upon stirring, breaks down into a heavy liquid. |

However, after heating at high temperatures some aerogel greases tend to lose consistency upon stirring. This is undesirable because there are many field applications where a grease is agitated or worked while subject to a high temperature and it is important that the grease retain its consistency under these conditions and subsequent thereto.

Accordingly, it is an object of the present invention to provide an aerogel grease having improved stability at high temperatures, particularly after working at high temperatures.

In accordance with the invention, these objects are accomplished by incorporating a water-miscible or water-soluble ether having at least two polar groups, of which at least one is an ether group and one at most is a hydroxyl or amine group, in an aerogel grease composition comprising a lubricating oil thickened with a non-abrasive, inorganic thickening or gelling agent, and particularly finely-divided silica, a silica aerogen being illustrative. The thickened lubricant so prepared has excellent temperature susceptibility properties.

The grease is also rendered more or less resistant to deterioration by water by incorporating a hydrophobic cationic surface-active wafer stabilizer therein in the form of Amine "O," 1-β-hydroxyethyl-2-heptadecenyl imidazoline.

The presence of the ether in an amount to obtain improved high temperature stability does not markedly affect the consistency of the thickened lubricant, i. e., the amount of the inorganic gelling agent to impart a given consistency to the thickened lubricant is not materially modified. Furthermore, the inclusion of the ether will not effect a change in the consistency of the thickened

lubricant upon storage. The ether likewise does not affect the water-resistance imparted to the grease by the hydrophobic cationic surface-active water stabilizing agent.

5 Due to the inorganic nature of the gelling agent, the thickened lubricant has excellent storage stability. This is to be contrasted with the heat susceptibility and deterioration of fatty materials in soap-base greases.

The preparation of the grease is simple and readily 10 adaptable to continuous operation, as contrasted with the involved grease-making techniques which are often considered in the industry as an art.

The oil stock used in making the thickened lubricant may be widely varied, as contrasted with present grease-making requirements in which the oil in many cases must 15 meet certain critical specifications.

In addition, the avoidance of the use of soap permits the manufacturer to be independent of the fat supply, which is important in periods in which fats and soaps are 20 scarce and, many times, of pronounced non-uniformity.

The inorganic gelling agent to be used in making the thickened lubricant in accordance with this invention may be any inorganic material which forms a gel with a lubricating oil and which is so finely-divided as to be 25 non-abrasive. The preferred materials are the aerogels, which may be formed from any material not incompatible with oil, such as silica, alumina, and other gel-forming metal oxides.

A series of silica aerogels which can be used as the in- 30 organic gelling agent of the invention are marketed under the trade name "Santocel."

Santocel C is prepared from a sodium silicate solution in the following way: The solution is neutralized with sulfuric acid and then allowed to stand until the mixture 35 sets to form a hydrogel. The byproduct sodium sulfate is washed out by the repeated washings with water. The continuous water phase in this hydrogel is then replaced by continued washing with alcohol until an alcogel is formed. In order to remove the liquid phase without a

40 collapse of the gel structure, the alcogel is placed in an autoclave which is then heated above the critical temperature of the alcohol and the pressure is allowed to increase to a point above the critical pressure of the alcohol. The vent valve is then opened and the alcohol allowed to 45 escape. Under these conditions, the silica gel structure remains practically undisturbed and the liquid phase of the gel is replaced with air. The material is then reduced in particle size by blowing it through a series of pipes containing sharp bends with jets of compressed air. 50 Santocel C has a secondary agglomerate particle size of about 3 to 5 microns.

Santocel A is prepared as set forth for Santocel C up to the point of removal of the product from the autoclave. This material is run through a continuous heating chamber where it is heated for ½ hour to a temperature of about 1500° F. to eliminate the last traces of volatile material. It is then broken down in a reductionizer or micronizer to a particle size of about  $\frac{1}{16}$  inch in diameter. The solids content of the original hydrogel used in preparing Santocel C is approximately 25% higher than that of Santocel A.

AR is a modification of A, differing only in that the material is reductionized to about the same particle size as C, approximately 1 to 6 microns in diameter.

65 ARD is a modification of AR, differing only in that ARD is densified by extracting air under vacuum, and therefore has a smaller volume than AR.

AX is an A which has not been devolatilized.

CDv is a C which has been devolatilized as set forth for A. CDv is reductionized before being devolatilized.

CDvR differs slightly from CDv in that the CDvR has been devolatilized just after heating in the autoclave and

then reductionized. It differs from CDv in that the latter is reductionized before being devolatilized.

The primary differences between the A's and the C's are as follows:

(1) The C's are prepared from a sodium silicate solution containing 25% more silica than the A's. Therefore, in general the A's are lighter and composed of smaller particles than the C's.

(2) The A's have undergone a devolatilization step in their preparation.

The following are the bulk densities of preferred silica aerogels:

|     | Density, grams per ml. |
|-----|------------------------|
| AR  | 0.029                  |
| ARD | 0.056 to 0.064         |
| C   | 0.082                  |

In general, AR and ARD show superior gelling ability and the A's in general are better than the C's. Silica aerogels which have been devolatilized generally have a higher gelling efficiency than the undevolatilized aerogels.

Other types of inorganic gelling agents which may be used include fumed silica. It is finely-divided and appears very much like an aerogel. It is made by a combustion or vaporization process, as a source of white "carbon black" for the rubber industry. The particles are several microns in size and porous in nature.

Another material is "Linde Silica Flour." It is very similar in physical appearance to the silica aerogel. The particle size of the silica is purported to be 0.01 to 0.05 micron and to be manufactured by burning silicon tetrachloride and collecting the combustion product on cool plates analogous to the production of carbon black. The particles are thought to be aggregates or clusters of particles rather than of sponge-like character.

Still another inorganic gelling agent known is "Ludox" silica which is known as a silica sol, and silica derivatives thereof. It has a particle size of the order of 0.01 to 0.03 micron.

In preparing thickened lubricants it is necessary to remove the water from the sol and replace it with an oil. This is possible by formulating the lubricant and removing the water by flash distillation or azeotropic distillation.

No attempt is made to enumerate all of the inorganic gelling agents which will be suitable, nor to present examples of all of them since the novel aspects of the invention reside in imparting high temperature stability to the lubricant rather than the use of novel gelling agents, per se.

The lubricating oil to be used in the process may have any lubricating viscosity. It may be raw oil, acid-refined, or solvent-refined, as required for the particular lubricating need.

The nature of the base oil has been found to make little difference in the relative consistencies of the thickened lubricants and conventionally (acid) refined oils produce slightly thicker lubricants than solvent-refined oils. Excellent working stability is obtained regardless of the type of the base oil. An increase in the viscosity of the base oil, as might be expected, brings increased viscosity to the thickened lubricant and minimizes bleeding. The change is relatively small and fairly linear. The viscosity of the oil does not affect the working stability of the lubricant.

The relative proportions of the inorganic gelling agent and the oil will vary somewhat depending upon the desired body in the thickened lubricant, the gelling ability of the inorganic gelling agent and the viscosity of the oil used. It has been noted, for instance, that with the Linde Silica Flour, the lubricants are somewhat harder, i. e., have a lower penetration than lubricants containing the same weight of Santocel. Lubricants made with low viscosity oils require a somewhat larger amount of the inorganic gelling agent to give a lubricant of the same penetration. The thickened lubricant may vary in consistency from the consistency of a slightly thickened oil to a solid or

semi-solid of grease-like consistency. In general, the amount of the inorganic gelling agent falls within the range of 5 to 20%, and in most cases would fall within the range of 7 to 12%.

The amount of the inorganic gelling agent, as might be expected, affects the consistency of the thickened lubricant in that an increase in its concentration brings a corresponding increase in consistency. The range is fairly linear and the amount of the gelling agent can be selected with relation to the consistency desired in view of the information in the following examples. While the difference is slight, the lubricants made with lower concentrations of gelling agent possess better working stability, while lubricants with larger amounts of gelling agent show slightly improved temperature susceptibility characteristics. The bleeding tendencies are decreased by increasing concentrations of the gelling agent.

In general, the properties of the thickened lubricants are remarkably independent of the composition variables and are not critical. The relative concentration of the gelling agent effects the most significant alteration, particularly with regard to the final consistency of the product. This permits the manufacture of thickened lubricants having a wide variety of consistencies.

A wide variety of water-miscible or water-soluble ethers (which can be regarded as ethers of polyhydric alcohols having  $n$  hydroxyl groups in which  $n$  or  $n-1$  hydroxyl groups of the polyhydric alcohol are etherified) can be employed in accordance with the invention to improve the high temperature stability of aerogel-base greases. Ethers which are water-immiscible, i. e., are oleaginous in character, cannot be used, because they are hydrophobic. The ether must be hydrophilic, for reasons which will be apparent from the theory of the action of the ether, set forth later. One hydroxyl or amino group increases the hydrophilic character of the ether.

The ether has from four to twenty carbon atoms and must contain at least two polar groups, of which at least one must be an ether group, one can be an amino group, and one can be a hydroxyl group. The ether can contain a mixture of ether groups with one amino and/or one hydroxyl group. It may contain as many as ten polar groups, those having two and three polar groups being most available and therefore being preferred. The latter ethers are employed in the examples because of their low cost and availability. The ethers in addition to one hydroxyl group and one amino group can contain inert substituents, such as halogen, which have been found not to reduce the activity of the compounds. Exemplifying

compounds within the scope of the invention are monoethyl ether of diethylene glycol, glycerol  $\alpha$ -hydroxy dimethyl ether, ethylene glycol monomethyl ether, monoethyl ether of triethylene glycol, diethylene glycol monomethyl ether, dimethoxy tetraethylene glycol, polymeric monohydroxyalkyl ethers of polyethers derived by condensation of ethylene oxide or propylene oxide, containing from two to ten oxide units, diethylene glycol monobutyl ether, diethylene glycol diethyl ether, monomethyl ether of glycerol chlorhydrin, ethylene glycol dimethyl ether tetraethylene glycol, and  $\beta,\beta'$ -diaminodiethyl ether.

The ether need not be oil-soluble, but should be oil-dispersible. It should have a minimum boiling point of about 150° C. since its primary purpose is to stabilize the grease at high temperatures.

The ether is incorporated in the aerogel-base grease in an amount to impart high temperature stability to the grease. Ordinarily, a concentration of ether ranging from 0.25 to about 1% by weight of the aerogel-base grease gives satisfactory results. There is no reason to employ more ether than is necessary, but excessive amounts do no harm, and amounts up to 5% or even higher have been successfully employed.

The amount of hydrophobic cationic surface-active agent to impart water-resistance to the aerogel grease in the form of 1- $\beta$ -hydroxyethyl-2-heptadecenyl imidazoline

will vary from 0.1% to about 5%, depending upon the water stabilizing effect desired, the amount and nature of the gelling agent used, and the economics involved.

In some instances, the composition containing the ether high temperature stabilizer may not display a long life when used continuously at high temperatures. A breakdown in high temperature stability at high temperatures if it appears is due to a decomposition, through oxidation, of the ether stabilizer of the invention. In such circumstances, it is desirable to include in the composition an antioxidant for the ether stabilizer. Conventional amine antioxidants which are more readily oxidized than the ethers of the invention can be employed for this purpose. Tetramethyldiaminodiphenylmethane, available under the trade name "Calco MB," is a particularly desirable antioxidant for the ethers of the invention. Only small quantities are required, and ordinarily an amount ranging from 0.1 to about 1% by weight of the aerogel base grease is ample. There is no reason to employ more antioxidant than is necessary to produce the desired effect, but excessive amounts do no harm and amounts up to 5% can be used, if desired.

The composition is made simply by mixing the inorganic gelling agent, the oil, the ether, the cationic water stabilizer and the antioxidant in any order or manner.

In one embodiment, the ether, the cationic water stabilizer and, desirably, the antioxidant, can be incorporated with the inorganic gelling agent either by mixing directly or, if desired, by dissolving them in a volatile hydrocarbon solvent, such as pentane, adding oil, mixing the solution with the inorganic gelling agent, and then evaporating the solvent.

Generally, the ether, the cationic water stabilizer and, optionally, the antioxidant are dispersed in the oil and the inorganic gelling agent added thereto and mixed therewith. Any simple mixing technique can be employed and, if desired, the mixture can be homogenized in a colloid mill, although this is not necessary.

The composition of the invention is not limited to the oil, gelling agent, cationic water stabilizer, and ether. Any of the materials conventionally added to lubricants and greases can be included. The expression "consisting essentially of" as used herein is intended to refer to the components which are essential to the composition, namely, the oil, the inorganic gelling agent and the ether, and the expression does not exclude other components from the composition which do not render it unsuitable for lubrication, such materials being, for instance, the cationic water stabilizer, the antioxidant, high polymers to modify viscosity or viscosity index, materials to impart tackiness, lubricating solids such as graphite, antioxidant additives, corrosion inhibitors of various types, sulfur, additives to render the lubricant suitable for use in gears, for cutting, grinding, etc.

The following examples illustrate preferred embodiments of the invention. In the examples, water-resistant thickened lubricants are prepared to show the absence of an effect of the ether on the water resistance of the grease.

#### Examples 1 to 4

Aerogel water-resistant greases of the following formulae were made up:

|                                      | A       | B       |
|--------------------------------------|---------|---------|
|                                      | Percent | Percent |
| Santocel A.R.D.                      | 8.0     | 8.0     |
| Amine "O" <sup>1</sup>               | 0.8     | 0.8     |
| Paratae <sup>2</sup>                 | 1.0     | 1.0     |
| Paraflo <sup>3</sup>                 | 0.5     | 0.5     |
| Methane base (Calco MB) <sup>4</sup> | 0.5     | 0.5     |
| Bright stock (78 SSU at 210° F.)     | 89.2    | 88.2    |
| Ether                                | 1.0     |         |

<sup>1</sup> 1-β-hydroxyethyl-2-heptadecenyl imidazoline.

<sup>2</sup> An isobutylene polymer sold by the Enjay Company, Inc. and commonly used in compounding greases.

<sup>3</sup> A Friedel-Crafts reaction product, useful as a pour point depressant and sold by the Enjay Company, Inc.

<sup>4</sup> Tetramethyldiaminodiphenylmethane.

Formula A is called the "Aerogel W. R. (Water-Resistant) Base Formula" (Example 2) in the table which follows. Example 1 is Formula A, without the Amine "O" and with 0.8% more of the base oil instead. Formula B is the water-resistant formula modified by addition of 1% ether in accordance with the invention (and reducing the Bright stock accordingly) in order to prepare an aerogel grease which is not only water-resistant but also stable at high temperatures.

In preparing these greases, the Amine "O" and the ether to be tested were dissolved in a stock solution of the base oil containing the other components. The Santocel was added to this solution and completely wetted by stirring. The grease was prepared at 95° F. by mixing for the time indicated in the following table, the time being varied so as to approximate the final penetration of the aerogel water-resistant base formula. If this time is the same as or longer and/or if the original penetration is the same as or less than that of the base formula, it is evident that the ether has either no or a beneficial effect on a yield.

The grease is prepared for the determination of high temperature stability by placing approximately 100 cc. of grease in a 150 ml. beaker. The beakers are heated to the test temperature by placing them in an aluminum block furnace. This furnace consisted of a solid block of aluminum heated by internal electrical heaters. Six holes, each large enough to accommodate a 150 cc. beaker, were drilled in the top of the block, together with a thermocouple, so that a measure of the temperature of the block could be obtained. In this manner, six beakers could be heated simultaneously. The beakers containing the grease were placed in the aluminum furnace and held there until the equilibrium temperature of the grease was 400° F. The samples were stirred at five-minute intervals during heating. After this the grease was allowed to cool to room temperature overnight and then was stirred vigorously with a spatula. The penetration of the grease was taken before and after heating in the block described in accordance with the Shell Microcone Penetration Test (Institute Spokesman (NLGI), VI, 12, page 1 (1943)).

TABLE II

| Ex. No. | Additive                                    | Mixing time, minutes | Immed. Shell pen. | No. cycles | High temperature stability—Shell penetration |            | Water stability |
|---------|---------------------------------------------|----------------------|-------------------|------------|----------------------------------------------|------------|-----------------|
|         |                                             |                      |                   |            | Initial                                      | Final      |                 |
| 1       | Aerogel base formula. <sup>1</sup>          | { 40<br>2 40 }       | 159               | { 5<br>5 } | 157<br>157                                   | 202<br>202 | None.<br>Do.    |
| 2       | Aerogel W. R. base formula. <sup>2</sup>    | { 30<br>2 30 }       | 159               | { 4<br>4 } | 171<br>171                                   | 267<br>267 | Good.<br>Do.    |
| 3       | Dimethoxytetraethylene glycol. <sup>3</sup> | { 30<br>2 30 }       | 121               | { 7<br>7 } | 126<br>178                                   | 219<br>210 | Do.<br>Do.      |
| 4       | do <sup>4</sup>                             | 30                   | 140               | 3          | 140                                          | 165        | None.           |

<sup>1</sup> No Amine "O"; contains 0.8% more base oil instead.

<sup>2</sup> Using a two-quart sample.

The results show that incorporating the Amine "O" in the aerogel base formula appreciably increases the penetration and thus reduces the high temperature stability. This effect of the Amine "O" is, however, overcome by the ethers added to the aerogel water-resistant base formula (Example 2). The data for Example 3 using the two-quart test demonstrates that the ether additive is still effective in large-scale preparations for both high temperature and water stabilization.

7  
Examples 5 to 15

A number of aerogel greases were prepared of the following formulations:

|                                      | A       | B       |
|--------------------------------------|---------|---------|
|                                      | Percent | Percent |
| Santocel ARD                         | 8.0     | 8.0     |
| Amine "O" <sup>1</sup>               | 0.8     | 0.8     |
| Paratac <sup>2</sup>                 | 1.0     | 1.0     |
| Paraflo <sup>3</sup>                 | 0.5     | 0.5     |
| Methane base (Calco MB) <sup>4</sup> | 0.5     | 0.5     |
| Bright stock (78 SSU at 210° F.)     | 89.2    | 88.2    |
| Ether                                |         | 1.0     |

<sup>1</sup> 1-β-hydroxyethyl-2-heptadecenylimidazoline.

<sup>2</sup> An isobutylene polymer sold by the Enjay Company, Inc. and commonly used in compounding greases.

<sup>3</sup> A Friedel-Crafts reaction product, useful as a pour point depressant and sold by the Enjay Company, Inc.

<sup>4</sup> Tetramethylidiaminodiphenylmethane.

Formula A is Example 5 in the table which follows. Formula B is the water-resistant formula of Formula A, modified by addition of 1% ether in accordance with the invention, reducing the Bright stock accordingly, in order to prepare an aerogel grease which is not only water-resistant but also stable at high temperatures.

In preparing these greases, the Amine "O" and the ether to be tested were dissolved in a stock solution of the base oil containing the other components. The Santocel was added to the solution and completely wetted by stirring. The grease was prepared at 95° F. by mixing for approximately twenty to thirty minutes, the time being adjusted to approximate the original penetration of Formula A.

The penetration of the grease was taken before and after heating in the block described in Example 1 in accordance with the Shell Micropenetration Test. After the data had been taken for four successive cycles, the average change in penetration per cycle was noted. The water stability of the greases was also determined. The following results were obtained:

TABLE III

| Ex. No. | Additive                            | Percent | "Block" test, Shell pens. |     |     |     |     | Δ pen./cycle | Water stability  |
|---------|-------------------------------------|---------|---------------------------|-----|-----|-----|-----|--------------|------------------|
|         |                                     |         | Orig.                     | 1st | 2nd | 3rd | 4th |              |                  |
| 5(a)    | Control with Amine "O"              |         | 139                       | 200 | 226 | —   | —   | 43.5         | Good.            |
| 5(b)    | do <sup>1</sup>                     |         | 171                       | —   | —   | —   | 267 | 24           | Do.              |
| 6       | Ethylene glycol monoethyl ether     | 1.0     | 150                       | 183 | 200 | 208 | —   | 19           | Do.              |
| 7       | Diethylene glycol monoethyl ether   | 1.0     | 149                       | 153 | 175 | 183 | —   | 11           | Do.              |
| 8(a)    | Diethylene glycol monoethyl ether   | 1.0     | 124                       | 160 | 169 | 186 | 189 | 16           | Do. <sup>1</sup> |
| 8(b)    | do <sup>1</sup>                     | 2.0     | 187                       | —   | —   | —   | 200 | 1.9          | Do. <sup>1</sup> |
| 9       | Diethylene glycol monobutyl ether   | 1.0     | 140                       | 199 | 197 | 215 | —   | 25           | Do.              |
| 10      | Diethylene glycol monoethyl ether   | 1.0     | 150                       | 174 | 203 | 204 | —   | 18           | Do.              |
| 11(a)   | Diethylene glycol diethyl ether     | 1.0     | 123                       | 146 | 176 | 190 | —   | 22           | Do.              |
| 11(b)   | do <sup>1</sup>                     | 2.0     | 193                       | —   | —   | —   | 220 | 4.3          | Do.              |
| 12(a)   | Diethylene glycol dibutyl ether     | 1.0     | 123                       | 154 | 188 | 193 | —   | 23           | Do.              |
| 12(b)   | do <sup>1</sup>                     | 2.0     | 182                       | —   | —   | —   | 214 | 8            | Do.              |
| 13      | Triethylene glycol monoethyl ether  | 1.0     | 154                       | 173 | 191 | 198 | —   | 15           | Do.              |
| 14      | Tetraethylene glycol dimethyl ether | 1.0     | 129                       | 157 | 168 | 185 | 193 | 16           | Do.              |
| 15(a)   | Tetraethylene glycol dibutyl ether  | 1.0     | 138                       | 154 | 192 | 199 | —   | 20           | Do.              |
| 15(b)   | do <sup>1</sup>                     | 2.0     | 193                       | —   | —   | —   | 240 | 11.8         | Do.              |

<sup>1</sup> Tested using a 2-quart sample.

The results show that incorporating the ether in the control grease (containing Amine "O" but no ether) appreciably increases high temperature stability, as evidenced by a reduction in penetration increase. This is best observable in the change in penetration per cycle noted in the above table. Diethylene glycol monomethyl ether and triethylene glycol monoethyl ether are most effective, but even the least effective of the additives gives a significant improvement in high temperature stability. The supplemental data in which two-quart samples were tested for Examples 8, 11, 12 and 15 shows that the ethers are effective for both high temperature and water stabilization, even in large-scale preparations.

## Examples 16 to 25

A number of aerogel greases were prepared as follows: A fixed quantity of oil (78 SSU at 210° F. solvent-extracted Bright stock) was weighed out into a 400 ml.

beaker. 0.8% Amine "O" was added, and 1% of the ether additive was incorporated in the base oil. The oil mix was heated to 130° F. while being mixed with a Lightnin' stirrer, and 8% Santocel ARD was mixed in with hand stirring. The resulting grease was allowed to stand overnight. An original penetration was then obtained using the Shell Microcone Penetration Test and the grease was then subjected to the block test. Grease samples exhibiting some degree of high temperature stability were cycled three or four times. Each sample was tested also for water stability and given a visual rating for consistency while at 400° F.

The ether additives tested included monohydroxy and nonhydroxy ethers. Several monohydric alcohols were included to compare the results obtainable. Data from these tests are given in the following table:

TABLE IV

| Ex. No. | Additive                          | "Block" test—Shell penetrations |     |     |     |     | Water stability |
|---------|-----------------------------------|---------------------------------|-----|-----|-----|-----|-----------------|
|         |                                   | Orig.                           | 1   | 2   | 3   | 4   |                 |
| 16      | Aerogel W. R. base formula.       | 139                             | 200 | 226 | —   | —   | Good.           |
| 17      | 2-ethylhexanol                    | 128                             | 290 | —   | —   | —   | Do.             |
| 18      | Lauryl alcohol                    | 135                             | 298 | —   | —   | —   | Do.             |
| 19      | 5-ethylnonanol-2                  | 156                             | 299 | —   | —   | —   | Do.             |
| 20      | Heptadecanol                      | 123                             | 269 | —   | —   | —   | Do.             |
| 21      | Cetyl alcohol                     | 126                             | 298 | —   | —   | —   | Do.             |
| 22      | Ethers                            | 150                             | 183 | 200 | 208 | —   | Do.             |
| 23      | Ethylene glycol monoethyl ether   | 124                             | 160 | 169 | 186 | 189 | Do.             |
| 24      | Diethylene glycol monoethyl ether | 140                             | 199 | 199 | 189 | 215 | Do.             |
| 25      | Diethylene glycol monobutyl ether | 120                             | 157 | 168 | 185 | 193 | Do.             |
|         | Dimethoxytetraethylene glycol     | —                               | —   | —   | —   | —   | —               |

Without exception, the five monohydric alcohols tested were unsatisfactory under high temperature conditions. The importance of an ether linkage is shown by comparison of these results with Examples 22, 23 and 24. The initial penetrations for diethylene glycol monoethyl ether and dimethoxytetraethylene glycol (Examples 23 and 25) are lower than that of the control grease, and indicate that these compounds have no deleterious effect on grease yield. The other ethers tested, Examples 22 and 24, also exert a stabilizing effect at high temperatures.

## Examples 26 and 27

Additional greases were prepared from a blend of Bright stocks to produce an oil of approximately 2000 SSU at 100° F. High temperature instability of aerogel greases is aggravated when a heavy base oil is used, and thus this provides a severe test of the high temperature stabilizing effect of the additives of the invention.

The test greases were prepared as outlined in the preceding Examples 16 to 25. The results are given in the following table:

TABLE V

| Ex. No. | Additive                           | "Block" test—Shell penetrations |     |     |     | Consistency (hot) | Water stability |
|---------|------------------------------------|---------------------------------|-----|-----|-----|-------------------|-----------------|
|         |                                    | Orig.                           | 1   | 2   | 3   |                   |                 |
| 26...   | Diethylene glycol monoethyl ether. | 163                             | 188 | 194 | 196 | Softer...         | Good.           |
| 27...   | Dimethoxytetraethylene glycol.     | 158                             | 182 | 186 | 196 | ...do....         | Do.             |

It is evident that the ethers are capable of increasing high temperature stability, even when a heavy base oil is employed.

In the examples, the high temperature stability of the aerogel greases is tested by heating the greases to 400° F. This is an extreme test, inasmuch as the highest temperature to which a grease is subjected under even extraordinary conditions of use is about 300° F., but it was adopted as a suitable test standard by which to measure the high temperature stability of the greases because a grease stable at 400° F. will definitely have the stability necessary to withstand heating to 300° F. It will be understood that for normal purposes an aerogel grease need not be stable at temperatures above about 300° F., and that the greases of the invention at least meet this requirement. Where the term "high temperature stability" is used, it will be understood to mean that the aerogel grease is stable at at least 300° F.

The following hypothesis is given as a partial explanation of the reason to which is attributed the action of the ether in improving the high temperature resistance of aerogel grease, but the invention is not to be bound thereby.

Silica aerogels are known to be in the form of an extremely finely-divided material and it is thought that it is capable of forming a colloidal structure in the oil vehicle employed in an aerogel grease. Mixing or stirring in formulating the grease serves to disperse the secondary aerogel agglomerates throughout the body of the oil. The aerogel occupies a greater volume than the liquid oil vehicle, and because of this it is probable that the colloidal structure is aided somewhat by a close packing of the solid silica gel particles perhaps with mechanical interlocking. It is thought that the basis of the structure is a tying together of the various silica aerogel particles by hydrogen bonding between hydroxyl groups which remain attached to individual silicon atoms in the silica gel molecule.

In setting up the colloidal grease structure, it is postulated that the distances between adjacent hydroxyl groups on different particles of silica aerogel may be too great in some circumstances to form a binding, attractive force between particles. In this event, water, which is always present in the aerogel structure, serves to bridge the gap between adjacent particles through hydrogen bonding between the compound and the hydroxyl groups on the adjacent silica aerogel particles. Thus the water in effect aids in setting up the colloidal grease structure, and may also link it together, at least in part.

When the grease under static conditions is submitted to temperatures high enough to volatilize the water no apparent effect is noticed at first, for there is no force to disarrange the structure. Consequently, penetration

vs. temperature curves indicate that aerogel greases have excellent high temperature performance with a very low increase in consistency as the temperature is increased. However, when this static state is disturbed by stirring, the structure can and does collapse, due to the absence of the water which has been volatilized and which formerly served as the connecting links between adjoining silica particles. In consequence, the structure passes from a gel state to a colloidal sol state. This explains why the transformation of the heated aerogel grease from a grease-like condition to a soupy condition occurs only after stirring and why stirring thus brings about an apparently irreversible gel-to-sol transformation. This transformation may be reversed to some extent by adding water to the soupy grease, tending to substantiate this hypothesis, but it is not possible to return the grease to its original condition.

Thus, on the basis of this hypothesis, incorporation in the grease, in accordance with the invention, of an ether which has at least two polar groups and which is not volatile at the temperatures to which the grease may be subjected leads to a partial or complete displacement of water in the aerogel by ether, possibly before and in any event at the time water is volatilized at an elevated temperature. The involatility of the ether prevents its loss during heating and thus prevents destruction of the colloidal grease structure when the aerogel grease is stirred after it has been heated to high temperatures. It is also apparent from this that a hydrophobic ether which is immiscible with water could not function in this way because it could not act as a substitute for water in the hydrophilic gel structure.

This application is a continuation-in-part of applications Serial Nos. 119,752, filed October 5, 1949 and 253,984, filed October 30, 1951, both now abandoned.

We claim:

1. A water-resistant thickened lubricant of good temperature susceptibility properties, consisting essentially of a mineral lubricating oil of lubricating viscosity, an inorganic water-sensitive gelling agent imparting a grease-like consistency to the oil upon addition thereto, 1- $\beta$ -hydroxyethyl-2-heptadecenyl imidazoline imparting stability against deterioration by water, and a water-soluble ether having a boiling point of at least 150° C. at atmospheric pressure and having at least two polar groups and imparting high temperature stability, at least one of which is an ether group, and one at most is selected from the group consisting of hydroxyl and amino groups.
2. A water-resistant thickened lubricant of good temperature susceptibility properties in accordance with claim 1 wherein the ether is diethylene glycol monoethyl ether.
3. A water-resistant thickened lubricant of good temperature susceptibility properties in accordance with claim 1 wherein the ether is dimethoxytetraethylene glycol.
4. A water-resistant thickened lubricant of good temperature susceptibility properties in accordance with claim 1 wherein the ether is ethylene glycol monoethyl ether.

#### 60 References Cited in the file of this patent

##### UNITED STATES PATENTS

|           |                  |               |
|-----------|------------------|---------------|
| 2,531,440 | Jordan           | Nov. 28, 1950 |
| 2,554,222 | Stross           | May 23, 1951  |
| 2,563,606 | Kimberlin et al. | Aug. 7, 1951  |
| 2,573,650 | Peterson         | Oct. 30, 1951 |
| 2,662,056 | McCarthy         | Dec. 8, 1953  |
| 2,675,148 | Iler             | Apr. 20, 1954 |
| 2,711,393 | Hughes et al.    | June 21, 1955 |